

## UNITED STATES PATENT OFFICE

2,419,360

## LUBRICATING OIL COMPOSITION

John G. McNab, Cranford, N. J., Carroll J. Wilson, Norwalk, Conn., and Carl Winning, Westfield, N. J., assignors to Standard Oil Development Company, a corporation of Delaware

No Drawing. Application December 21, 1944,  
Serial No. 569,258

15 Claims. (Cl. 252—42.7)

1

This invention relates to lubricating oils and methods for preparing the same, and more particularly to mineral lubricating oil compositions for use as crankcase lubricants in internal combustion engines.

This application is a continuation-in-part of our co-pending application Serial No. 425,129, filed December 31, 1941.

Because in recent years the requirements for lubricating oils for gasoline and Diesel engines have steadily been made more stringent, it has been proposed to add various ingredients to these oils to improve their behavior in such service. One purpose of these ingredients is to impart detergency to the oils, thus bringing about greater engine cleanliness and avoiding ring sticking, carbon formation and varnish deposition. Certain of these ingredients also impart oxidation resistant properties to oils, thereby tending to inhibit the development of corrosive ingredients in such oils. Corrosion-preventing addition agents are particularly required when the oil is to come in contact with the newer type of alloys of silver and cadmium and of copper and lead, which are now widely used as bearing metals.

It has been found that the addition of small amounts of metal derivatives of organic compounds, such as metallic phenolates, alcoholates, enolates, etc., imparts special detergent properties to such oils, by which the deposition of varnish, sludge and other oil deterioration products on engine parts is prevented and such engine parts are maintained in a high degree of cleanliness. Unfortunately, on account of their metallic content, these compounds generally increase the corrosiveness of the oil to some extent, although in some cases they retard the corrosiveness to a minor degree. It has been proposed to add sulfur, nitrogen or phosphorus compounds to offset the corrosive action of the metallic compounds, but these additives tend to react with the metallic compounds to impair engine cleanliness and to permit more corrosion than would have been anticipated.

Moreover, in the use of metallic phenolates, alcoholates and the like the effectiveness of these compounds is gradually spent. The detergent capacity becomes exhausted as deterioration products, soot, dirt, varnish, etc., accumulate in the lubricant and saturate the adsorptive power of the additive. In engines equipped with a filter, the latter tends to remove the additive, particularly when the additive is adsorbed on contamination products which are strained out by the filter. The oxidation processes which are underway in

2

an oil during use operate upon the antioxidant functions of the additive and thus also contribute to its exhaustion. The oxidation of the oil also creates insoluble substances which the detergent is called upon to adsorb, thus lessening its capacity for dispersing contamination products which enter the oil, and acidic substances are also formed which may react directly with the detergent to destroy its efficacy. When the detergent is employed also to impart corrosion resistant properties to the oil, the above degradation phenomena all hasten to break down this corrosion resistance.

It has now been found, in accordance with the present invention, that, by adding to the lubricating oil containing phenolates, alcoholates and the like a second additive comprising the product obtained by alkylating p-cresol with a tertiary alkyl group, the corrosiveness of the oil will be greatly retarded and at the same time the cleanliness of the engine will be found to be even greater than when the metallic compound is used alone. The second compound also affords protection against corrosion even after the detergent has become saturated with dispersed materials or removed by an oil filter.

The metallic derivatives of organic compounds which may be successfully used in combination with the new class of ether additives may be defined by the formula

## ROM

Where R is an aromatic or aliphatic radical and M is any metal or other basic acting unit, such as a basic radical, but is preferably a metal selected from groups I, II, III, IV, and VIII of the periodic table. In this class of compounds the oxygen is attached to a carbon atom which is in turn attached only to carbon, hydrogen or nitrogen. Where M is polyvalent, the additional valences of M may be joined to other similar RO— groups or to other organic groups or inorganic constituents. This class of compounds includes not only the metal phenolates, alcoholates, enolates, etc., but also the metal naphtholates and other similar compounds containing more than one benzene nucleus as well as compounds in which one or more hydrogen atoms of the organic radical are substituted with alkyl, aryl, hydroxyl, nitro, amino, imino, or other groups, or substituent atoms such as halogen. It is essential, however, that the compound employed should not contain a carboxyl group attached to carbon in an aliphatic chain, lest, on hydrolysis, an acid strong enough to attack en-

gine parts, despite the presence of the stabilizing compound, be generated. In place of the metals there may be substituted basic radicals, such as ammonium or the various onium groups, such as the quarternary ammonium base radicals or the corresponding sulfonium, phosphonium and similar radicals.

The preferred groups of compounds falling within the above defined class are the phenolates, alcoholates and enolates of metals of groups I, II, III, IV or VIII. Typical examples of these compounds are the following:

*A. Alcoholates.*—General formula  $ROM$ , where  $R$  is an aliphatic or substituted aliphatic or non-benzenoid cyclic radical:

Calcium cetylate,  $Ca(C_{12}H_{25}O)_2$   
Calcium octadecylate,  $Ca(C_{18}H_{37}O)_2$   
Barium octadecylate,  $Ba(C_{18}H_{37}O)_2$   
Zinc chlorohexadecylate,  $Zn(C_{16}H_{32}ClO)_2$   
Barium tert.-octyl benzylate,



Tin salt of wax alcohols,  $(CH_3(CH_2)_nCH_2O)_2Sn$   
Magnesium salt of naphthenic alcohols

*B. Phenolates.*—General formula  $ROM$ , where  $R$  is an aromatic or substituted aromatic radical:

Tin tert.-octyl phenolate,



Calcium iso-dodecyl naphtholate,



Barium p-tert.-amyl phenolate,



Barium salt of phenols derived from oil of cashew nut shells (having an unsaturated  $C_{14}$  side chain).

Calcium salts of petroleum phenols.

*C. Enolates.*—General formula



where  $R$  and  $R'$  are organic groups:

Calcium salt of hexyl acetoacetic acid ester,



Barium salt of butyl acetoacetic acid ester,



Tin salt of oleyl methyl ketone,



Cobalt salt of amyl benzoyl acetone,



Calcium salt of stearophenone,



Barium oleyl amide,



With regard to the alkylated phenolates used in this invention, the alkyl radicals should be of sufficient size to impart adequate oil solubility to the compounds and such alkyl radicals as butyl, amyl, tert.-octyl, decyl, cetyl, and stearyl have been found satisfactory. Whenever the tert.-octyl group is mentioned in this specification, the tetramethylbutyl radical, formed by polymerizing isobutylene, is meant.

When the phenolic groups are alkylated with petroleum olefinic hydrocarbons, such as refinery gases and the like, the resulting products may comprise a mixture of compounds with different sizes of alkyl groups.

In some cases the phenolic compounds may be alkylated with long chain groups such as those derived from petroleum wax or an ester wax. In such cases one wax group may be attached to each aryl group or several aryl groups may be attached to one wax group at several points along the chain, as represented below.

50        
55        
60        
65        
70        
75        
80        
85        
90        
95        
100       
105       
110       
115       
120       
125       
130       
135       
140       
145       
150       
155       
160       
165       
170       
175       
180       
185       
190       
195       
200       
205       
210       
215       
220       
225       
230       
235       
240       
245       
250       
255       
260       
265       
270       
275       
280       
285       
290       
295       
300       
305       
310       
315       
320       
325       
330       
335       
340       
345       
350       
355       
360       
365       
370       
375       
380       
385       
390       
395       
400       
405       
410       
415       
420       
425       
430       
435       
440       
445       
450       
455       
460       
465       
470       
475       
480       
485       
490       
495       
500       
505       
510       
515       
520       
525       
530       
535       
540       
545       
550       
555       
560       
565       
570       
575       
580       
585       
590       
595       
600       
605       
610       
615       
620       
625       
630       
635       
640       
645       
650       
655       
660       
665       
670       
675       
680       
685       
690       
695       
700       
705       
710       
715       
720       
725       
730       
735       
740       
745       
750       
755       
760       
765       
770       
775       
780       
785       
790       
795       
800       
805       
810       
815       
820       
825       
830       
835       
840       
845       
850       
855       
860       
865       
870       
875       
880       
885       
890       
895       
900       
905       
910       
915       
920       
925       
930       
935       
940       
945       
950       
955       
960       
965       
970       
975       
980       
985       
990       
995       
1000       
1005       
1010       
1015       
1020       
1025       
1030       
1035       
1040       
1045       
1050       
1055       
1060       
1065       
1070       
1075       
1080       
1085       
1090       
1095       
1100       
1105       
1110       
1115       
1120       
1125       
1130       
1135       
1140       
1145       
1150       
1155       
1160       
1165       
1170       
1175       
1180       
1185       
1190       
1195       
1200       
1205       
1210       
1215       
1220       
1225       
1230       
1235       
1240       
1245       
1250       
1255       
1260       
1265       
1270       
1275       
1280       
1285       
1290       
1295       
1300       
1305       
1310       
1315       
1320       
1325       
1330       
1335       
1340       
1

pirical formula  $C_{15}H_{24}O$ , and a melting point of about  $69.2-69.4^{\circ} C$ . The same product may be obtained by reacting p-cresol with tertiary butyl alcohol. In this case the amount of sulfuric acid catalyst is preferably quite large, i. e., of the order of one mol of catalyst per mol of p-cresol. Temperatures from about  $0^{\circ} C$ . to about  $50^{\circ} C$ . may be used, preferably from  $25^{\circ}$  to  $40^{\circ} C$ .

The lubricating oil base stocks of this invention may be straight mineral lubricating oils or distillates derived from paraffinic, naphthenic, asphaltic or mixed base crudes, or, if desired, various blended oils may be employed as well as residuals, particularly those from which asphaltic constituents have been carefully removed. The oils may be refined by conventional methods using acid, alkali and/or clay or other agents such as aluminum chloride, or they may be extracted oils produced, for example, by solvent extraction with solvents of the type of phenol, sulfur dioxide, furfural, dichloro ethyl ether, propane, nitrobenzene, crotonaldehyde, etc. Hydrogenated oils or white oils may be employed as well as synthetic oils prepared, for example, by the polymerization of olefins or by the reaction of oxides of carbon with hydrogen or by the hydrogenation of coal or its products. In certain instances cracking coal tar fractions and coal tar or shale oil distillates may also be used. Also, for special applications, animal, vegetable or fish oils or their hydrogenated or volatilized products may be employed, either alone or in admixture with mineral oils.

For the best results, however, the base stock chosen should usually be that oil which without the additive present gives the optimum performance in the service contemplated. Since one advantage of the additives is that their use also makes feasible the employment of less satisfactory mineral oils or other oils, no strict rule can be laid down for the choice of the base stock. Certain essentials must of course be observed. The oil must possess the viscosity and volatility characteristics known to be required for the service contemplated. The oil must be a satisfactory solvent for the additive, although in some cases auxiliary solvent agents may be used. The lubricating oils, however they may have been produced, may vary considerably in viscosity and other properties depending upon the particular use for which they are desired, but they usually range from about 40 to 150 seconds Saybolt viscosity at  $210^{\circ} F$ . For the lubrication of medium and high speed Diesel engines the general practice has been to use a lubricating oil base stock prepared from naphthenic or aromatic crudes and having a Saybolt viscosity at  $210^{\circ} F$ . of 45 to 90 seconds and a viscosity index of 0 to 50. However, in certain types of Diesel service, and in gasoline engine service, oils of higher viscosity index are often required, for example, up to 75 or 100, or even higher, viscosity index.

In addition to the materials to be added according to the present invention, other agents may also be used such as dyes, pour depressors, heat thickened fatty oils, sulfurized fatty oils, organo metallic compounds, metallic or other soaps, sludge dispersers, antioxidants, thickeners, viscosity index improvers, oiliness agents, resins, rubber, olefin polymers, volatilized fats, volatilized mineral oils, and/or volatilized waxes and colloidal solids such as graphite or zinc oxide, etc. Solvents and assisting agents, such as esters, ketones, alcohols, aldehydes, halogenated or nitrated compounds, and the like, may also be employed.

Assisting agents which are particularly desir-

able are the higher alcohols having eight or more carbon atoms and preferably 12 to 20 carbon atoms. The alcohols may be saturated straight and branched chain aliphatic alcohols such as octyl alcohol,  $C_8H_{17}OH$ , lauryl alcohol,  $C_{12}H_{25}OH$ , cetyl alcohol,  $C_{16}H_{33}OH$ , stearyl alcohol, sometimes referred to as octadecyl alcohol,  $C_{18}H_{37}OH$ , and the like; the corresponding olefinic alcohols such as oleyl alcohol; cyclic alcohols, such as naphthenic alcohols; and aryl substituted alkyl alcohols, for instance, phenyl octyl alcohol, or octadecyl benzyl alcohol or mixtures of these various alcohols, which may be pure or substantially pure synthetic alcohols. One may also use mixed naturally occurring alcohols such as those found in wool fat (which is known to contain a substantial percentage of alcohols having about 16 to 18 carbon atoms) and in sperm oil (which contains a high percentage of cetyl alcohol); and although it is preferable to isolate the alcohols from these materials, for some purposes the wool fat, sperm oil or other natural products rich in alcohols may be used per se. Products prepared synthetically by chemical processes may also be used, such as alcohols prepared by the oxidation of petroleum hydrocarbons, e. g., paraffin wax, petrolatum, etc.

Generally the amount of each of the additives of the present invention in the finished lubricant composition should be between the approximate limits of 0.02 and 2.0%, and preferably from 0.1 to 1.0%, the exact amount to be used depending to a certain extent on the particular compounds used, the character of the mineral oil base and the operating conditions of the engine in which the lubricant is to be used.

Compositions in which two or more metal compounds are used with one or more of the p-cresol reaction products or in which one metal compound is used with two or more of the p-cresol reaction products are also contemplated in this invention.

The following example shows the effect of the use of a p-cresol alkylation product upon the corrosion of a copper-lead bearing when used in combination with various metallic compounds of the class defined above, when compared with the results obtained with oils containing the metal compound only. Included is an example of the use of a calcium soap as the detergent compound instead of a metallic phenolate, alcoholate or similar compound, showing that the new class of corrosion inhibiting additives cannot advantageously be used with all types of detergents.

#### Example 1

Samples of oil blends containing, separately, the metal compounds of the present invention as the sole additive and the same compounds in combination with a p-cresol alkylation product, were submitted to a bearing corrosion test in which the extent of weight loss of the bearings due to corrosion by the oils was determined. This test was conducted as follows:

500 cc. of the oil was placed in a glass oxidation tube (13" long and 2 1/2" diameter) fitted at the bottom with a 1/4" bore air inlet tube perforated to facilitate air distribution. The oxidation tube was then immersed in a heating bath so that the oil temperature was maintained at  $325^{\circ} F$ . during the test. Two quarter sections of automotive bearings of copper-lead alloy of known weight having a total area of 25 sq. cm. were attached to opposite sides of a stainless steel rod which was then immersed in the test oil and

rotated at 600 R. P. M., thus providing sufficient agitation of the sample during the test. Air was then blown through the oil at the rate of 2 cu. ft. per hour. At the end of each four-hour period fresh bearings were supplied and 15% of the oil in the oxidation tube was removed and a corresponding amount of fresh oil blend was added. Each time the bearings were removed they were washed with naphtha and weighed to determine the amount of loss by corrosion. The cumulative weight losses of all the bearings used in a given test at the end of the various four-hour periods are given in Table 1.

Table 1

| Oil                                                              | Cumulative Bearing Weight Loss, mg. |        |         |         |
|------------------------------------------------------------------|-------------------------------------|--------|---------|---------|
|                                                                  | 4 Hrs.                              | 8 Hrs. | 12 Hrs. | 16 Hrs. |
| (A) Refined mineral lubricating oil (S. A. E. 20)                | 1                                   | 252    | —       | —       |
| (B) Oil A + 1.0% calcium octadecylate                            | 70                                  | —      | —       | —       |
| (C) Oil B + 0.25% additive M <sup>1</sup>                        | 1                                   | 3      | 36      | —       |
| (D) Oil A + 1.0% calcium salt of hexyl ester of acetoacetic acid | 0                                   | 2      | 39      | —       |
| (E) Oil D + 0.25% additive M <sup>1</sup>                        | 0                                   | 1      | 1       | 4       |
| (F) Oil A + 0.3% barium salt of cashew nut shell phenol          | 2                                   | 16     | 235     | —       |
| (G) Oil F + 0.25% additive M <sup>1</sup>                        | 1                                   | 6      | 20      | —       |
| (H) Oil A + 0.2% calcium erucate                                 | 34                                  | —      | —       | —       |
| (J) Oil H + 0.25% additive M <sup>1</sup>                        | 88                                  | —      | —       | —       |

<sup>1</sup> Product obtained by reacting p-cresol with isobutene.

It will be noted from the data given in Table 1 that addition of calcium octadecylate made the mineral lubricating oil more corrosive but that when the p-cresol reaction product was added to the compounded oil the resulting blend was even less corrosive than the mineral oil alone. Blends containing a calcium enolate (Oil D) and a barium phenolate (Oil F) were somewhat less corrosive than the mineral oil itself, but in each case the corrosiveness was still further minimized when the additive was added to the blends (Oils E and G). On the other hand, when the p-cresol reaction product was added to an oil blend containing a calcium soap of a carboxylic acid (Oil H), the corrosiveness was increased rather than decreased (Oil J).

In addition to being employed in crankcase lubricants for Diesel and automotive engines, the additives of the present invention may also be used in light mineral oils such as spindle oils and textile oils, metal cutting oils, turbine oils, insulating and transformer oils, steam cylinder oils and greases. Also, since these additives achieve their detergent effect by modifying surface activity, their use in asphalt, road oils and waxes to improve wetting and adhesive properties is also contemplated. Likewise, they may be added to liquid fuels to increase their wetting ability for metals, enabling them to displace moisture which might otherwise cause corrosion of containers, fuel lines, pump parts, and the like.

This invention is not to be considered as limited by any theory of the action of the various additives nor by any of the examples mentioned or described herein which are given for illustrative purposes only, but it is to be limited solely by the terms of the appended claims.

We claim:

1. An organic composition containing a small quantity, sufficient to impart detergent properties, of an organic compound of the formula

ROM

where R is a member of the group consisting of

aliphatic and aromatic radicals which are free from carboxyl and metal substituted carboxyl groups, M is a member of the class consisting of metals and basic radicals, and the oxygen is attached to a carbon atom which is attached only to carbon, hydrogen or nitrogen, and a small quantity, at least sufficient to offset the corrosive effect of the first-named compound, of a product obtained by reacting para-cresol with a reagent which furnishes a tertiary alkyl group, in the presence of an alkylation catalyst.

2. An improved lubricant which comprises an oil base, a small quantity, sufficient to impart detergent properties, of an organic compound of the formula

ROM

where R is a member of the class consisting of aliphatic and aromatic radicals which are free from carboxyl and metal substituted carboxyl groups, M is a basic acting unit, and the oxygen is attached to a carbon atom which is attached only to carbon, hydrogen or nitrogen, and a small quantity, at least sufficient to offset the corrosiveness of the first-named compound, of a product obtained by reacting para-cresol with a reagent which furnishes a tertiary alkyl group, in the presence of an alkylation catalyst.

3. A lubricant for internal combustion engines which comprises a mineral oil base, a small quantity, sufficient to impart detergent properties, of a compound of the formula

ROM

where R is a member of the class consisting of aliphatic and aromatic radicals which are free from carboxyl and metal substituted carboxyl groups, M is a metal of Group II of the Periodic Table, and the oxygen is attached to a carbon atom which is attached only to carbon, hydrogen or nitrogen, and a small quantity, at least sufficient to offset the corrosiveness of the first-named compound, of a product obtained by reacting para-cresol with a reagent which furnishes a tertiary alkyl group, in the presence of an alkylation catalyst.

4. A lubricant for internal combustion engines which comprises a mineral oil base, a small quantity, sufficient to impart detergent properties, of a compound of the formula

ROM

where R is a member of the group consisting of aliphatic and aromatic radicals which are free from carboxyl and metal substituted carboxyl groups, M is a metal of Group II of the Periodic Table, and the oxygen is attached to a carbon atom which is attached only to carbon, hydrogen or nitrogen, and a small quantity, at least sufficient to offset the corrosiveness of the first-named compound, of the product obtained by reacting para-cresol with isobutene in the presence of an alkylation catalyst.

5. A lubricant for internal combustion engines which comprises a mineral oil base, a small quantity, sufficient to impart detergent properties, of a metallic alcoholate and a small quantity, at least sufficient to offset the corrosiveness of the said metallic alcoholate, of a product obtained by reacting para-cresol with a reagent which furnishes a tertiary alkyl group, in the presence of an alkylation catalyst.

6. A lubricant for internal combustion engines which comprises a mineral oil base, a small quantity, sufficient to impart detergent properties, of

a metallic enolate which is free from carboxyl and metal substituted carboxyl groups, and a small quantity, at least sufficient to offset the corrosiveness of the said metallic enolate, of a product obtained by reacting para-cresol with a reagent which furnishes a tertiary alkyl group, in the presence of an alkylation catalyst.

7. A lubricant for internal combustion engines which comprises a mineral oil base, a small quantity, sufficient to impart detergent properties, of a metallic phenolate which is free from carboxyl and metal substituted carboxyl groups and a small quantity, at least sufficient to offset the corrosive tendency of the said metallic phenolate, of a product obtained by reacting para-cresol with a reagent which furnishes a tertiary alkyl group, in the presence of an alkylation catalyst.

8. A lubricant for internal combustion engines which comprises a mineral oil base, a small quantity, sufficient to impart detergent properties, of calcium octadecylate and a small quantity, at least sufficient to offset the corrosiveness of the said calcium octadecylate, of the product obtained by reacting para-cresol with isobutene in the presence of a catalytic amount of sulfuric acid.

9. A lubricant for internal combustion engines which comprises a mineral oil base, a small quantity, sufficient to impart detergent properties, of the barium salt of cashew nut shell phenol, and a small quantity, at least sufficient to offset the corrosiveness of the said barium salt, of the product obtained by reacting para-cresol with isobutene in the presence of a catalytic amount of sulfuric acid.

10. A lubricant for internal combustion engines which comprises a mineral oil base, a small quantity, sufficient to impart detergent properties, of the calcium salt of the hexyl ester of acetoacetic acid, and a small quantity, at least sufficient to offset the corrosiveness of the said calcium salt, of the product obtained by reacting para-cresol with isobutene in the presence of a catalytic amount of sulfuric acid.

11. A lubricant for internal combustion engines which comprises a mineral oil base, 0.02% to 2.0% of a compound of the formula ROM where R is a member of the group consisting of aliphatic and aromatic radicals which are free from carboxyl and metal substituted carboxyl groups, M is a metal, and the oxygen is attached to a carbon atom which is attached only to carbon, hydrogen or nitrogen, and 0.02% to 2.0% of the product obtained by reacting para-cresol with isobutene in the presence of sulfuric acid as a catalyst at a temperature of about 70° C.

12. A lubricant for internal combustion engines which comprises a mineral oil base, a small quantity, sufficient to impart detergent properties, of a compound of the formula ROM where R is a member of the group consisting of aliphatic and aromatic radicals which are free from carboxyl and metal substituted carboxyl groups, M is a metal of Group II of the Periodic Table, and the oxygen is attached to a carbon atom which is attached only to carbon, hydrogen or

nitrogen, and a small quantity, at least sufficient to offset the corrosive effect of the first-named compound, of the product obtained by reacting para-cresol with isobutene in the presence of sulfuric acid as a catalyst, said product having a molecular weight of about 220, a chemical composition corresponding to the empirical formula  $C_{15}H_{24}O$ , and being, when purified, a white crystalline solid having a melting point of about 69.2-69.4° C.

13. A lubricant for internal combustion engines which comprises a mineral oil base, a small quantity, sufficient to impart detergent properties, of calcium octadecylate, and a small quantity, at least sufficient to offset the corrosiveness of the said calcium octadecylate, of the product obtained by reacting para-cresol with isobutene in the presence of sulfuric acid as a catalyst, said product having a molecular weight of about 220, a chemical composition corresponding to the empirical formula  $C_{15}H_{24}O$ , and being, when purified, a white crystalline solid having a melting point of about 69.2-69.4° C.

14. A lubricant for internal combustion engines which comprises a mineral oil base, a small quantity, sufficient to impart detergent properties, of the barium salt of cashew nut shell phenol, and a small quantity, at least sufficient to offset the corrosiveness of the said barium salt, of the product obtained by reacting para-cresol with isobutene in the presence of sulfuric acid as a catalyst, said product having a molecular weight of about 220, a chemical composition corresponding to the empirical formula  $C_{15}H_{24}O$ , and being, when purified, a white crystalline solid having a melting point of about 69.2-69.4° C.

15. A lubricant for internal combustion engines which comprises a mineral oil base, a small quantity, sufficient to impart detergent properties, of the calcium salt of the hexyl ester of acetoacetic acid, and a small quantity, at least sufficient to offset the corrosiveness of the said calcium salt, of the product obtained by reacting para-cresol with isobutene in the presence of sulfuric acid as a catalyst, said product having a molecular weight of about 220, a chemical composition corresponding to the empirical formula  $C_{15}H_{24}O$ , and being, when purified, a white crystalline solid having a melting point of about 69.2-69.4° C.

JOHN G. McNAB.  
CARROLL J. WILSON.  
CARL WINNING.

## REFERENCES CITED

55 The following references are of record in the file of this patent:

## UNITED STATES PATENTS

| Number    | Name                   | Date          |
|-----------|------------------------|---------------|
| 2,362,293 | McNab et al. -----     | Nov. 7, 1944  |
| 2,361,051 | Patterson et al. ----- | Oct. 24, 1944 |
| 2,346,808 | Winning et al. -----   | Apr. 18, 1944 |
| 2,294,145 | Winning et al. -----   | Aug. 25, 1942 |
| 2,248,830 | Stillson et al. -----  | July 8, 1941  |
| 2,202,825 | Brandes -----          | June 4, 1940  |